

## UNITED STATES PATENT OFFICE

1,984,203

HARD METALLIC COMPOSITION AND  
CONTACTS THEREOF

George N. Sieger, Indianapolis, Ind., assignor to  
P. R. Mallory & Co., Incorporated, Indianapolis,  
Ind., a corporation of Indiana

No Drawing. Application December 12, 1931,  
Serial No. 580,729

12 Claims. (Cl. 200—166)

This invention relates to a hard metallic composition, the method of making the same and electrical make-and-break contacts formed therefrom and, more particularly, to a composition of 5 a hard refractory metal carbide and silver, the method of forming such a composition and electrical make-and-break contacts formed from such a composition.

General objects of the invention are the provisions of such a hard metallic composition having improved electrical and physical characteristics, the improved method of forming the same and improved electrical make-and-break contacts formed from such composition which have 10 low surface contact resistance, high current carrying capacity and a minimum tendency to stick together during operation.

More specifically, objects of the invention are the provisions of such a composition of hard metal carbide and silver which has an electrical conductivity higher than that of compositions of tungsten and silver and which is comparable to that of pure silver, a high degree of malleability and physical characteristics which tend to insure 15 original shape and surface condition of elements of electrical apparatuses formed from such composition subjected to various types of forces in operation; and a novel method of forming such composition which preferably includes as one step 20 thereof the mixing of finely divided particles of a hard metal carbide and silver prior to the formation of bodies therefrom.

A further object of the invention is the provision 25 of such electrical make-and-break contacts formed from a material of a hard refractory metal carbide and silver which have a minimum tendency to oxidize and to transfer metal from one contact to a cooperating contact, a minimum internal resistance, low surface contact resistance 30 and a minimum surface resistance rise in operation.

Other objects of the invention will in part be 35 obvious and will in part appear hereinafter.

The invention accordingly comprises the several steps and the relation and order of one or more of such steps with respect to each of the others, the composition and the article possessing the features, properties, and the relation of constituents which are exemplified in the following detailed disclosure, and the scope of the application of which will be indicated in the claims.

The composition of the present invention is adapted for a variety of uses in electrical fields since it has a high electrical conductivity, a high 40 degree of malleability, is resistive to deformation

and deterioration under conditions which are encountered in the operations of many electrical apparatuses and which have been found to have deleterious effects on the compositions, alloys or metals recognized prior to the present invention as representing the best available materials. A hard metal carbide, and, more particularly, tungsten carbide has relatively no malleability, a low degree of electrical conductivity and a high melting point. Silver added to the carbide will provide 5 the desired electrical conductivity and malleability. Such a composition primarily consists of a mass of a hard metal carbide and silver dispersed throughout the mass providing electrical conductive paths therethrough. Silver wets hard metal carbides and thus remains thoroughly bound 10 within the mass of carbide under conditions normally deformative and/or destructive to silver bodies.

The percentage of silver in this hard metallic 15 composition may vary widely, such as from a few per cent to an amount such that the composition contains a relatively small amount of hard metal carbide, dependent upon the characteristics desired. The malleability and electrical conductivity are increased by an increase in the amount 20 of silver. When high percentages of silver are used the mass of hard metal carbide must be highly porous to provide sufficient voids to receive the silver. If a porous base is formed from 25 the hard metal carbide prior to the incorporation of silver many difficulties are encountered in obtaining a rigid body having the required porosity. These difficulties are overcome by the practice of 30 the improved method described herein whereby 35 at least some of the silver is incorporated with the hard metal carbide prior to the formation of bodies or slugs or the composition.

Prior to the present invention the use of electrical make-and-break contacts in various fields 40 has given rise to many problems, the chief of which are high surface contact resistance, low current carrying capacity, high contact resistance in comparison with the resistance of the remaining portions of an electrical circuit, tendency of the contacts to fuse and stick together 45 during operation, high rate of oxidation of contact surfaces, high rate of transfer from one contact to another, high internal resistance, high rate of surface resistance rise and many other 50 problems.

In accordance with the present invention, it has been found that generally enhanced characteristics can be imparted to electrical apparatus and make-and-break contacts which are de- 55

signed for use in fields where low surface contact resistance and high current carrying capacity are necessary; where the use of small contacts, the resistance of which in itself must be low in comparison with that of the other portions of the circuit, is desired; where the tendency of cooperating contacts to fuse and stick together must be kept to a minimum; in resistance welding; and, more specifically in relays; 5 in circuit breakers; and, in interrupters for welders, by using in their formation a hard metallic composition comprising, in its preferred form, tungsten carbide and silver.

The ingredients and proportions used in the 15 electrical make-and-break contact composition of the present invention are subject to variations within reasonable limits, that is, for example, the silver may vary between about 20 per cent and about 70 per cent of the contact composition, the 20 balance being tungsten carbide. However, the preferred proportions of the ingredients are as follows:

|                     | Per cent |
|---------------------|----------|
| 25 Tungsten carbide | 40       |
| Silver              | 60       |

In accordance with the preferred method of forming the composition of the present invention, the tungsten carbide is formed by any well 30 recognized method, reduced to powdered form, and mixed with finely divided particles of silver. The resultant mixture is pressed into porous slugs which are then sintered and subjected to fused silver which will run throughout the porous structure, impregnation being abetted by 35 capillary action.

Within the range of percentages of silver given above the double addition method of the addition of silver is preferred since it insures a high percentage of silver in the resultant composition. 40 However, it has been found possible when using relatively low percentages of silver within that range to impregnate the porous slugs of tungsten carbide directly with silver without first reducing the former to a powdered form and mixing there- 45 with a portion of the silver. When, however, high percentages of silver are desired it has been found that the percentage of voids in the porous slugs of tungsten carbide is such as to allow only a portion of the desired amount of silver to be impregnated therein directly. Thus a certain percentage of the silver is added to the tungsten carbide in the manner described above prior to the impregnation of the porous slugs with silver. The 50 chief factors governing the percentage range of silver for electrical make-and-break contacts are internal resistance and physical hardness. Below 20 per cent of silver, the composition is found to have an undesirably high internal resistance and above 70 per cent of silver the composition is found to be too soft for many contact purposes. The preferred composition of the material is given above as comprising 40 per cent tungsten carbide and 60 per cent silver.

Following the preferred method the composition having the preferred proportions of ingredients set forth above is preferably produced by mixing about 55 per cent of tungsten carbide powder with about 45 per cent powdered silver metal. This mixture is preferably prepared by ball milling the tungsten carbide and silver powder for a considerable period of time, such as, for example, about 3 hours in a mill containing clean steel balls. After the mixing is completed, the material is preferably paraffined with a solu- 70

tion of paraffin and carbon tetrachloride and thoroughly dried to volatilize the carbon tetrachloride. Sufficient paraffin solution is used such that the resultant mixture of tungsten carbide, silver and paraffin contains about 1 per cent paraffin which is used to insure freedom from cracks due to pressing. The resultant mixture is then pressed into porous slugs, preferably at a pressure of about 2 tons per square inch. The resultant slugs are then preferably subjected to a sintering process which, among other functions, serves to remove the paraffin, and impregnated with the remaining portion of silver preferably during the sintering process, about 45 per cent by weight of pure silver preferably in 15 the form of shot being placed adjacent the porous slugs in a suitable furnace and the whole being heated to a temperature of about 1350° C. It is obvious, however, that the invention may be practiced by first sintering slugs of tungsten carbide and silver and then impregnating the resultant porous slugs with the remaining portion of the silver. 20

For the purposes of the present invention tungsten is the preferred hard refractory metal, 25 although other similar metals of the same group and sub-group of Mendelejeff's periodic table, such as molybdenum, which for some purposes prove satisfactory, are contemplated. The tungsten carbide gives to the composition made 30 in accordance with the present invention a desired rigidity and resistance to deformation not present in electrical make-and-break contacts formed from pure silver. In addition, it provides a retaining base for the silver constituent which 35 thoroughly wets the former. This base retains the silver in a particularly characteristic dispersed manner such that temperatures which will fuse contacts of pure silver, allowing the latter to stick together and deform during 40 operation, will have no deleterious effect upon electrical make-and-break contacts of the present invention. The silver in the composition insures a high current carrying capacity and low internal resistance in addition to various other 45 characteristics which may be attributed to this constituent.

Without attributing all of the desirable characteristics of the composition of the present invention to either one or the other of the specific 50 constituents, it is found that the composition, the method of making the same, and electrical make-and-break contacts made therefrom in accordance with the teachings of the present invention attain the objects set forth above in an 55 admirable and efficient manner.

Since certain changes in carrying out the above process and certain modifications in the composition and article which embody the invention may be made without departing from its scope, 60 it is intended that all matter contained in the above description shall be interpreted as illustrative and not in a limiting sense.

It is also to be understood that the following claims are intended to cover all of the generic 65 and specific features of the invention herein described, and all statements of the scope of the invention which, as a matter of language, might be said to fall therebetween.

Having described my invention, what I claim 70 as new and desire to secure by Letters Patent, is:

1. An electrical make-and-break contact comprising a composition produced by forming a porous mass of silver and a carbide of one of the 75

hard refractory metals molybdenum and tungsten and incorporating in the pores of said porous mass a binding constituent of silver, the silver in said composition constituting from about 20 to 5 70 per cent thereof.

2. An electrical make-and-break contact comprising from about 20 to 70 per cent silver and the balance of a carbide of one of the hard refractory metals molybdenum and tungsten, said contact being formed by impregnating with a mass of molten silver the pores of a porous mass consisting of silver binding together particles of the refractory metal carbide and having a greater electrical conductivity than a contact formed 10 from silver and the hard refractory metal with the amount of silver in the latter equal to the amount of silver in the former.

3. An electrical make-and-break contact comprising from about 20 to 70 per cent silver and the balance of tungsten carbide, said contact being formed by impregnating with a mass of molten silver the pores of a porous mass consisting of silver binding together particles of tungsten carbide and having a greater electrical conductivity than a contact formed from silver and tungsten with the amount of silver in the latter equal to the amount of silver in the former.

4. An electrical make-and-break contact comprising about 40 per cent tungsten carbide and about 60 per cent silver.

5. The method of producing electrical make-and-break contact composition comprising mixing finely divided particles of a hard refractory metal carbide and silver, pressing the mixture to form a slug, sintering the slug and impregnating the slug with silver.

6. The method of producing electrical make-

and-break contact composition comprising mixing finely divided particles of tungsten carbide and silver, pressing the mixture to form a porous slug, sintering the porous slug and impregnating the porous slug with silver.

7. The method of producing electrical make-and-break contact composition comprising mixing finely divided particles of a hard refractory metal carbide and silver, pressing the mixture to form a porous slug, placing a body of silver adjacent the porous slug in a furnace and heating to a temperature to cause the porous slug to be sintered and the body of silver to impregnate the porous slug.

8. The method of producing electrical make-and-break contact composition comprising mixing finely divided particles of tungsten carbide and silver, pressing the mixture to form a porous slug, placing bodies of silver adjacent the porous slug in a furnace and heating the whole to a sufficient temperature to cause the porous slug to be sintered and to fuse the bodies of silver to cause the silver to impregnate the porous slug.

9. An electrical make-and-break contact comprising from about 20 to 70 per cent of silver and the balance of tungsten carbide.

10. An electrical make-and-break contact composed of silver and tungsten carbide.

11. An electrical make-and-break contact composed of silver and molybdenum carbide.

12. An electrical make-and-break contact composed of a refractory metallic constituent and silver, said refractory metallic constituent comprising carbide of one of the refractory metals molybdenum and tungsten.

GEORGE N. SIEGER.